

(Model.)

S. H. HAMILTON.

MANUFACTURE OF PAPER BOARD.

No. 269,815.

Patented Dec. 26, 1882.

Fig. 1.



Fig. 2.



WITNESSES-

John Hutchinson.

Henry B. Hazard.

INVENTOR-

S. H. Hamilton, by  
Prindle & Co., his Atty.

# UNITED STATES PATENT OFFICE.

SILAS H. HAMILTON, OF BUSHNELL, ASSIGNOR, BY MESNE ASSIGNMENTS,  
TO MARVIN A. FARR, OF CHICAGO, ILLINOIS.

## MANUFACTURE OF PAPER-BOARD.

SPECIFICATION forming part of Letters Patent No. 269,815, dated December 26, 1882.

Application filed August 13, 1878. Renewed October 24, 1881. (Model.)

*To all whom it may concern:*

Be it known that I, SILAS H. HAMILTON, of Bushnell, in the county of McDonough, and in the State of Illinois, have invented certain new and useful Improvements in the Manufacture of Paper-Board; and I do hereby declare that the following is a full, clear, and exact description thereof, reference being had to the accompanying drawings, making a part of this specification, in which—

Figure 1 is a perspective view of my improved board, a portion of one edge being broken to show the manner of combining the sheets; and Fig. 2 is a cross-section of the same.

Letters of like name and kind refer to like parts in each of the figures.

The design of my invention is to render practicable the employment of paper as a substitute for wood for building and other like purposes, to which end it consists principally in an improved article of manufacture composed of paper-pulp, glue, and bichromate of potash mixed together, formed into sheets, and subjected to heavy rolling pressure, substantially as and for the purpose hereinafter specified.

It consists, further, in an improved article of manufacture consisting of a board composed of sheets of the before-named product which are caused to adhere together by means of pressure, substantially as and for the purpose hereinafter shown.

It consists, finally, in an improved article of manufacture consisting of paper-pulp, glue, bichromate of potash, alum, and silica, formed into sheets by pressure, substantially as and for the purpose hereinafter set forth.

In the use of my invention I take one and one-half ton of paper-pulp—preferably made from straw, cane, or other cheap material—forty-nine pounds of glue, and one and one-eighth pound of bichromate of potash, both in solution, and mix the same thoroughly, after which the composition is made into sheets A in the usual manner, except that said sheets are subjected to more than ordinary pressure between rollers. Two or more of the sheets

A are then coated exteriorly with a solution of glue and bichromate of potash, placed with their faces in contact, and then passed between pressure-rollers, which cause said sheets to become firmly united, after which, if de-

sired, the board B thus produced may be coated exteriorly with the solution named, 55 and then surfaced by means of calendered or plage pressure-rollers. When it is desired that the board B shall be fire-proof a solution composed of fifty pounds of alum and two pounds of soluble glass are added to the 60 above-named quantity of composition before the same is passed through the paper-machine. The glue operates primarily to cause the pulp to adhere firmly together, while the addition of the bichromate of potash causes 65 the whole to become water-proof.

While the proportions of ingredients before named are preferably employed, any other proportions deemed best may be used without departure from the spirit of my invention.

The article thus produced has no grain, is homogeneous and possesses in a marked degree durability and ability to resist abrasive wear, and, in addition thereto, is not affected 75 by heat or dampness, in consequence of which it is especially adapted for use in connection with the interior and exterior finish of buildings for residence or business purposes.

Having thus fully set forth the nature and 80 merits of my invention, what I claim as new is—

1. An improved article of manufacture composed of paper-pulp, glue, and bichromate of potash mixed together, formed into sheets, and 85 subjected to heavy rolling pressure, substantially as and for the purpose specified.

2. An improved article of manufacture consisting of a board composed of sheets of paper-pulp, glue, and bichromate of potash, 90 which sheets are caused to adhere together by means of pressure, substantially as and for the purpose shown.

3. An improved article of manufacture consisting of paper-pulp, glue, bichromate of potash, alum, and silica, mixed together and 95 formed into sheets by pressure, substantially as and for the purpose set forth.

In testimony that I claim the foregoing I have hereunto set my hand this 12th day of 100 August, 1878.

SILAS H. HAMILTON.

Witnesses:

GEO. S. PRINDLE,  
JAS. E. HUTCHINSON.